

## UNITED STATES PATENT OFFICE.

RALPH E. SAYRE, OF NEW ROCHELLE, NEW YORK, ASSIGNOR TO METALS RECOVERY COMPANY, OF NEW YORK, N. Y., A CORPORATION OF MAINE.

## CONCENTRATION OF ORES.

No Drawing.

Application filed November 28, 1923. Serial No. 677,580.

*To all whom it may concern:*

Be it known that I, RALPH E. SAYRE, a citizen of the United States, residing at New Rochelle, in the county of Westchester, 5 State of New York, have invented certain new and useful Improvements in the Concentration of Ores; and I do hereby declare the following to be a full, clear, and exact description of the invention, such as will 10 enable others skilled in the art to which it appertains to make and use the same.

This invention relates to the concentration of ores, minerals, and the like, by flotation, and has for its object the provision of 15 certain improvements in flotation processes, and more particularly the froth flotation processes.

The present invention is based upon the discovery that the salts of substituted 20 dithiocarbamic acids are effective flotation reagents, particularly in non-acid or alkaline pulps. I have found that the salts of substituted dithiocarbamic acids have a marked selective action on sulfide minerals, 25 as distinguished from gangue minerals, and when used as flotation agents in the customary flotation processes cause the sulfide mineral to float readily with an attendant high recovery of the metal values. My 30 investigations indicate that the salts of substituted dithiocarbamic acids are substantially lacking in frothing power, so that an appropriate frothing agent, such as pine-oil, terpineol, or the like, should be employed in conjunction therewith in carrying out the flotation operation.

The salts of substituted dithiocarbamic acids (dithiocarbamates) may be prepared in accordance with well-known methods. In 40 general, the most convenient procedure for preparing such salts consists in adding an alkali dissolved in alcohol to a mixture of carbon bisulfide and an amine. The aryl dithiocarbamates (for example, potassium phenyldithiocarbamate,  $C_6H_5NHS_2K$ ) may be prepared in this manner employing an arylamine. In preparing the alkyl dithiocarbamates (for example, diethylammonium diethyldithiocarbamate  $(C_2H_5)_2NCS_2NH_2$ , 45  $(C_2H_5)_2$ ) an alkylamine may be dissolved in benzene and treated with carbon bisulfide. In order to obtain the reaction product in solid form, it is usually desirable to treat the reaction mixture with ether or with 50 some other solvent in which the dithiocarba-

mate is but slightly soluble. It is not necessary for the purposes of the present invention to isolate the dithiocarbamate from the reaction mixture. Thus, in the practice of the present invention, the dithiocarbamates 60 may be used as crude reaction products without being isolated from the reaction mixture.

The alkali and alkylammonium salts of substituted dithiocarbamic acids are in general 65 readily soluble in water and alcohol. The heavy metal salts (such as the lead, zinc, iron etc. salts) may be obtained as precipitates by treating the dissolved dithiocarbamates (such as the alkali and alkyl-ammonium dithiocarbamates) with a dissolved salt of the heavy metal. Thus, for example, lead phenyl dithiocarbamate is produced by mixing solutions of lead acetate and potassium phenyl dithiocarbamate. In 75 general, the heavy metal dithiocarbamates are only sparingly soluble even in hot water.

I have found that while the alkyl dithiocarbamates possess marked flotation properties the aryl dithiocarbamates are even more 80 effective flotation agents, and for this reason I prefer, in carrying out the present invention, to use the aryl compounds.

In practicing the present invention, I have found that the readily soluble dithiocarbamates give the best results when introduced into the flotation circuit immediately before the flotation operation. The same procedure may be employed when using the less soluble dithiocarbamates, such 90 as the heavy metal dithiocarbamates, the salts being dissolved in hot water before being introduced into the flotation circuit. When using the heavy metal dithiocarbamates, I prefer, however, to add the sparingly soluble dithiocarbamates to the ore pulp prior to the final grinding operation.

The quantity of the dithiocarbamate to be employed in practicing the present invention depends to some extent upon the particular salt being used and the particular ore being treated. In general, I have found that one-fifth of a pound, and less, per ton of dry ore gives satisfactory results.

I prefer to employ the dithiocarbamates 105 as flotation agents in a neutral (that is non-acid) or alkaline pulp. Any alkali, such as caustic soda, soda ash, or lime, may be added to the ore pulp in order to make the pulp neutral or alkaline. Lime, on the whole, 110

is the most suitable and available alkali for this purpose. The alkali should be added to the ore pulp before the final grinding.

The dithiocarbamates are of some value as flotation agents in acid pulps, but the metallurgical results obtained by the use of these agents in acid pulps are by no means as good as those obtained in alkaline pulps. This is probably due in some part to the instability of the free dithiocarbamic acids, which are liberated from their salts by mineral acids.

In the following table, I have given some typical flotation results obtained in the practice of the present invention. In all of the floats reported in this table, 500 grams of a partially ground copper sulfide ore (of the Utah Copper Company), assaying 1.34% copper were ground for twenty minutes in a pebble mill with 250 c. c. of water and an amount of lime equivalent to four pounds per ton of dry ore. The flotation operation was carried out in a laboratory size Calow rougher cell, after diluting the ground ore pulp to about 2.5 liters. The lead, iron and zinc dithiocarbamates were added to the ore pulp at the start of the grinding operation, while the potassium dithiocarbamates were added after the grinding operation and immediately preceding the flotation operation. In each case a drop of the terpineol was added to the ore pulp immediately preceding flotation.

| 35 | Reagent.                             | Amount used per ton of ore. | Conc. copper. | Tailings copper. | Recovery  |
|----|--------------------------------------|-----------------------------|---------------|------------------|-----------|
|    |                                      | Pound.                      | Per cent.     | Per cent.        | Per cent. |
| 40 | Potassium phenyldithiocarbamate      | 0.2                         | 14.5          | 0.28             | 80.8      |
|    | Lead phenyldithiocarbamate           | 0.1                         | 15.5          | 0.26             | 83.2      |
|    | Potassium o-tolyldithiocarbamate     | 0.1                         | 14.1          | 0.32             | 77.9      |
|    | Iron o-tolyldithiocarbamate          | 0.1                         | 15.6          | 0.30             | 79.1      |
|    | Potassium a-naphthylidithiocarbamate | 0.1                         | 15.3          | 0.29             | 80.1      |
| 45 | Zinc a-naphthylidithiocarbamate      | 0.1                         | 18.4          | 0.33             | 76.8      |

It will be understood by those skilled in the art that the present invention is applicable to the treatment by flotation of various kinds of mineral mixtures both natural and artificial. In the appended claims I have accordingly employed the terms "mineral" and "ore" in a broad sense to include ores, mineral products and all materials amenable to concentration or similar treatment by the flotation processes.

I claim:

1. The improvement in the concentration

of minerals by flotation which comprises subjecting the mineral in the form of a pulp to a flotation operation in the presence of a dithiocarbamate.

2. The improvement in the concentration of minerals by flotation which comprises subjecting the mineral in the form of a pulp to a flotation operation in the presence of an aryl dithiocarbamate.

3. The improvement in the concentration of minerals by flotation which comprises subjecting the mineral in the form of a non-acid pulp to a flotation operation in the presence of a dithiocarbamate.

4. The improvement in the concentration of minerals by flotation which comprises subjecting the mineral in the form of a non-acid pulp to a flotation operation in the presence of an aryl dithiocarbamate.

5. The improvement in the concentration of minerals by flotation which comprises subjecting the mineral in the form of an alkaline pulp to a flotation operation in the presence of a dithiocarbamate.

6. The improvement in the concentration of minerals by flotation which comprises subjecting the mineral in the form of an alkaline pulp to a flotation operation in the presence of an aryl dithiocarbamate.

7. The improvement in the concentration of minerals by flotation which comprises subjecting the mineral in the form of a pulp made alkaline by the addition of lime to a flotation operation in the presence of an aryl dithiocarbamate.

8. The method of concentrating ores and the like which comprises subjecting the ore in the form of a suitable pulp to a flotation operation in the presence of a salt of a substituted dithiocarbamic acid.

9. The method of concentrating ores and the like which comprises subjecting the ore in the form of a suitable pulp to a flotation operation in the presence of a salt of a substituted dithiocarbamic acid which salt is only sparingly soluble in water.

10. The method of concentrating ores and the like which consists in subjecting the ore in the form of a suitable pulp to a flotation operation in the presence of a heavy metal salt of a substituted dithiocarbamic acid.

11. The method of concentrating ores and the like which consists in subjecting the ore in the form of a suitable pulp to a flotation operation in the presence of lead phenyldithiocarbamate.

In testimony whereof I affix my signature.

RALPH E. SAYRE.